



US008067318B2

(12) **United States Patent**  
**Martin**

(10) **Patent No.:** **US 8,067,318 B2**  
(45) **Date of Patent:** **Nov. 29, 2011**

(54) **ELASTIC NONWOVEN SHEET**

(75) Inventor: **Kenneth E. Martin**, Newark, DE (US)

(73) Assignee: **Invista North America S.a.r.l.**,  
Wilmington, DE (US)

(\*) Notice: Subject to any disclaimer, the term of this  
patent is extended or adjusted under 35  
U.S.C. 154(b) by 755 days.

(21) Appl. No.: **11/112,537**

(22) Filed: **Apr. 22, 2005**

(65) **Prior Publication Data**

US 2005/0239363 A1 Oct. 27, 2005

**Related U.S. Application Data**

- (63) Continuation-in-part of application No. 10/413,172,  
filed on Apr. 14, 2003, now Pat. No. 6,942,896.  
(60) Provisional application No. 60/372,911, filed on Apr.  
15, 2002, provisional application No. 60/565,014,  
filed on Apr. 23, 2004.

(51) **Int. Cl.**

*B32B 5/04* (2006.01)  
*C08J 5/24* (2006.01)  
*D04H 1/64* (2006.01)

(52) **U.S. Cl.** ..... **442/328; 442/105; 442/327; 427/496;**  
427/501

(58) **Field of Classification Search** ..... **442/59-180;**  
428/904

See application file for complete search history.

(56)

**References Cited**

**U.S. PATENT DOCUMENTS**

|             |   |         |                      |         |
|-------------|---|---------|----------------------|---------|
| 4,066,397 A | * | 1/1978  | Carroll .....        | 8/192   |
| 4,366,814 A |   | 1/1983  | Riedel et al.        |         |
| 4,443,513 A |   | 4/1984  | Meitner et al.       |         |
| 4,613,537 A | * | 9/1986  | Krupper .....        | 428/192 |
| 4,965,122 A |   | 10/1990 | Morman               |         |
| 4,981,747 A |   | 1/1991  | Morman               |         |
| 5,114,781 A |   | 5/1992  | Morman               |         |
| 5,244,482 A |   | 9/1993  | Hassenboehler        |         |
| RE35,206 E  |   | 4/1996  | Hassenboehler et al. |         |
| 5,910,224 A | * | 6/1999  | Morman .....         | 156/178 |

**FOREIGN PATENT DOCUMENTS**

|    |          |   |        |
|----|----------|---|--------|
| EP | 0472924  | * | 3/1992 |
| EP | 0472942  | * | 3/1992 |
| JP | 47-24479 |   | 7/1972 |

**OTHER PUBLICATIONS**

ASTM D 1117-77-97a Standard Test Methods for Nonwoven Fabrics.

\* cited by examiner

*Primary Examiner* — Angela Ortiz

*Assistant Examiner* — Jennifer Steele

(74) *Attorney, Agent, or Firm* — Christina W. Geerlof

(57) **ABSTRACT**

This invention relates to stretchable nonwoven sheets prepared by substantially uniformly impregnating a necked nonwoven substrate or an easily extensible as-made nonwoven substrate with an elastomeric polymer by treatment with an elastomeric polymer solution. The nonwoven sheet is useful in the manufacture of diapers and other hygiene articles.

**14 Claims, No Drawings**

## 1

## ELASTIC NONWOVEN SHEET

## CROSS-REFERENCE TO RELATED APPLICATIONS

This application claims priority from U.S. provisional application Ser. No. 60/565,014, filed Apr. 23, 2004. This application is also a continuation-in-part of U.S. patent application Ser. No. 10/413,172, filed Apr. 14, 2003 and now U.S. Pat. No. 6,942,896, which claims priority from U.S. provisional application Ser. No. 60/372,911, filed Apr. 15, 2002. All of these applications are incorporated herein by reference.

## BACKGROUND OF THE INVENTION

## 1. Field of the Invention

This invention relates to stretchable nonwoven sheets suitable for use in the manufacture of personal hygiene articles. More specifically, the stretchable nonwoven sheets are formed by substantially uniformly impregnating a necked nonwoven substrate or an easily extensible as-made nonwoven substrate with an elastomeric polymer.

## 2. Description of Related Art

Elastic nonwoven materials are well known in the art. Examples of elastic nonwoven materials include "stretch-bonded" and "neck-bonded" laminates. Stretch-bonded laminates are prepared by joining a gatherable layer to an elastic layer while the elastic layer is in an extended condition so that upon relaxing the layers, the gatherable layer is gathered. Neck-bonded laminates are produced by joining a necked, non-elastic layer with an elastic film on fiber layer. The elastic layer generally comprises an elastic film or an elastic nonwoven web. These elastic nonwoven laminates require the preparation of at least two separate nonwoven or film layers.

U.S. Pat. No. 4,366,814 to Riedel (Riedel) describes a breathable elastic bandage material comprising at least 50 weight percent of an extensible fabric capable of an elongation of at least 30% without tearing and at least 15 weight percent of an elastomer impregnated in the fabric without filling the holes in the fabric.

U.S. Pat. No. 5,910,224 to Morman (Morman) describes a method for making a stretchable composite by applying an elastomeric precursor to a neckable material such as a nonwoven web, neck stretching the neckable material and treating the elastomeric precursor, such as by heating, while the neckable material is in a necked condition to form an elastomeric layer bonded to the necked material. Preferred elastomeric precursors comprise a latex or a thermoset elastomer. The elastomeric precursor is applied to the neckable material in an amount between 5 g/m<sup>2</sup> to about 50 g/m<sup>2</sup>. The elastomeric layer typically penetrates the web from about 2 to about 10 fiber thicknesses and the degree of penetration of the elastomeric precursor is controlled so that there is no strikethrough to the side of the web opposite the side on which the elastomeric layer has been applied. The resulting stretchable composite therefore has a film-like hand on the side comprising the elastomeric layer and retains the original soft hand of the neckable material on the side opposite the elastomeric layer.

Published European Patent Application No. 0472942 describes an elastomeric saturated nonwoven material having a compressibility and recovery in the Z-direction which includes a fibrous web, such as a nonwoven web of meltblown fibers, that is saturated with a polymeric material, such as an elastomeric acrylic latex, polyurethane latex, or nitrile rubber latex.

## 2

Published Japanese Patent Application No. 47-24479 is directed to belts for use in conveyors and power transmissions that are made by impregnating needlepunched nonwoven fabrics with rubber or synthetic resins.

5 There is a continued need for elastic sheet materials that can be produced economically, have soft stretch and good holding power, and which have a fabric-like hand on both surfaces.

## 10 BRIEF SUMMARY OF THE INVENTION

The subject invention is directed to a method for forming a stretchable nonwoven sheet comprising the steps of:

15 providing a necked nonwoven substrate having a thickness, first and second outer surfaces, a machine direction and a cross-direction, the necked nonwoven substrate having a percent elongation of at least 30% in the cross-direction; substantially uniformly impregnating the necked nonwoven substrate with a solution comprising an elastomeric 20 polymer dissolved in a solvent; and

removing the solvent from the impregnated nonwoven substrate by wet coagulation to deposit the elastomeric polymer substantially uniformly throughout the thickness of the nonwoven substrate without forming a substantially continuous layer of elastomeric polymer on either of the first or second outer surfaces of the nonwoven substrate.

The subject invention is further directed to a method for forming a stretchable nonwoven sheet comprising the steps of:

30 providing an easily extensible as-made nonwoven substrate having a thickness, first and second outer surfaces, a machine direction and a cross-direction, a percent elongation of at least 30% in the cross-direction, a basis weight between about 15 g/m<sup>2</sup> and about 100 g/m<sup>2</sup>, a break tenacity greater than 500 g/in;

35 substantially uniformly impregnating the easily extensible as-made nonwoven substrate with a solution comprising an elastomeric polymer dissolved in a solvent; and

removing the solvent from the easily-extensible as-made nonwoven substrate by wet coagulation to deposit the elastomeric polymer substantially uniformly throughout the thickness of the nonwoven substrate without forming a substantially continuous layer of elastomeric polymer on either of the first or second outer surfaces of the nonwoven substrate.

45 The subject invention is also directed to a stretchable nonwoven sheet comprising a nonwoven substrate that has been necked in a necked direction and substantially uniformly impregnated with an elastomeric polymer, the stretchable nonwoven sheet having a ratio of third unload cycle force at 100% elongation to third load cycle force at 100% elongation, after the stretchable nonwoven sheet has been extended to 140% in the necked direction three times, of at least 0.3:1.

The subject invention is additionally directed to a stretchable nonwoven sheet comprising an easily extensible as-made nonwoven substrate that has been substantially uniformly impregnated with an elastomeric polymer, the stretchable nonwoven sheet having a ratio of third unload cycle force at 30% elongation to third load cycle force at 30% elongation, after the stretchable nonwoven sheet has been extended to 30% in the cross-direction three times, of at least 0.15:1.

## DETAILED DESCRIPTION OF THE INVENTION

In the current invention, a stretchable composite nonwoven sheet is provided by impregnating a necked nonwoven substrate or an easily extensible as-made nonwoven substrate with a solution comprising a solvent and an elastomeric poly-

mer. The necked nonwoven substrate or easily extensible as-made nonwoven substrate is impregnated under conditions that achieve substantially uniform impregnation of the nonwoven substrate without forming a polymer layer on either surface thereof. After removal of the solvent, a breathable impregnated nonwoven sheet is obtained which has an unexpected combination of high unload cycle force compared to load cycle force (for good holding power and soft stretch) in the cross-direction and a textile-like hand. Further, the inventive sheet is typically simpler to make and thinner than conventional multilayer stretch laminates. For example, the inventive sheet can have a typical thickness of about 0.25 mm to 0.75 mm, whereas stretch laminates are generally thicker than 1.3 mm.

The term "polymer" as used herein, generally includes but is not limited to, homopolymers, copolymers (such as for example, block, graft, random and alternating copolymers), terpolymers, etc. and blends and modifications thereof. Furthermore, unless otherwise specifically limited, the term "polymer" shall include all possible geometrical configurations of the material. These configurations include, but are not limited to isotactic, syndiotactic and random symmetries.

The term "polyester" as used herein is intended to embrace polymers wherein at least 85% of the recurring units are condensation products of dicarboxylic acids and dihydroxy alcohols with linkages created by formation of ester units. This includes aromatic, aliphatic, saturated, and unsaturated di-acids and di-alcohols. The term "polyester" as used herein also includes copolymers (such as block, graft, random and alternating copolymers), blends, and modifications thereof. A common example of a polyester is poly(ethylene terephthalate) (PET) which is a condensation product of ethylene glycol and terephthalic acid.

The term "polyurethane" as used herein is intended to include block copolymers made by condensing a difunctional polyol with a diisocyanate and a difunctional chain extender, as described in detail hereinbelow.

The term "polyolefin" as used herein, is intended to mean any of a series of largely saturated open chain polymeric hydrocarbons composed only of carbon and hydrogen. Typical polyolefins include, but are not limited to, polyethylene, polypropylene, polymethylpentene and various combinations of the ethylene, propylene, and methylpentene monomers.

The term "polyethylene" as used herein is intended to encompass not only homopolymers of ethylene, but also copolymers wherein at least 85% of the recurring units are ethylene units.

The term "polypropylene" as used herein is intended to embrace not only homopolymers of propylene but also copolymers where at least 85% of the recurring units are propylene units.

The term "elastomeric polymer" as used herein refers to any polymer that, when formed into a sheet, fiber, or film and upon application of a biasing force, is elongatable to a stretched length that is at least about 160 percent of its relaxed unbiased length and that will recover at least 55 percent of its elongation upon release of the elongating biasing force. For example, a one centimeter sample of material that is elongatable to at least 1.6 centimeters and which, upon being elongated to 1.6 centimeters by application of a force and with release of the force, will recover to a length of not more than 1.27 centimeters. Many elastomeric materials exist which may be stretched by much more than 60% of their relaxed length, for example 100 percent or more, and many of these will recover to substantially their original relaxed length, for

example, to within 105 percent of their original relaxed length, upon release of the stretching force.

The terms "nonwoven fabric" or "nonwoven web" as used herein mean a structure of individual fibers, filaments, or threads that are positioned in a random manner to form a planar material without an identifiable pattern, as opposed to a knitted or woven fabric.

The term "spunbond" filaments as used herein means filaments which are formed by extruding molten thermoplastic polymer material as filaments from a plurality of fine, usually circular, capillaries of a spinneret with the diameter of the extruded filaments then being rapidly reduced by drawing. Other filament cross-sectional shapes such as oval, multi-lobal, etc. can also be used. Spunbond filaments are generally continuous and have an average diameter of greater than about 5 micrometers. Spunbond nonwoven fabrics or webs are formed by laying spunbond filaments randomly on a collecting surface such as a foraminous screen or belt. Spunbond webs are generally bonded by methods known in the art, such as hot-roll calendering or passing the web through a saturated-steam chamber at an elevated pressure. Also, the web can be thermally point bonded at a plurality of thermal bond points located across the spunbond fabric.

The term "machine direction" (MD) is used herein to refer to the direction in which a nonwoven web is produced. The term "cross-direction" (XD) refers to the direction generally perpendicular to the machine direction.

The term "necking" as used herein refers to a method which involves applying a force to a nonwoven fabric, for example parallel to the machine direction of the nonwoven, to cause the nonwoven fabric to elongate in the direction the force is applied and to reduce its width in the direction perpendicular to that of the elongation, for example in the cross-direction, in a controlled manner to a desired amount. The direction perpendicular to the elongating force is referred to herein as the "necked direction". The controlled stretching and necking may take place at room temperature or at temperatures higher or lower than room temperature and is limited to an increase in overall dimension in the direction being stretched up to the elongation required to tear or break the fabric.

The terms "necked nonwoven fabric" and "necked nonwoven substrate" are used herein to refer to any nonwoven fabric which has been constricted in at least one direction by processes such as drawing. A "neckable nonwoven fabric" is a nonwoven fabric that can be constricted in at least one dimension in a necking process. The term "percent neckdown" refers to the ratio determined by measuring the difference between the un-necked dimension and the necked dimension (measured in the necked direction) and then dividing the difference by the un-necked dimension and multiplying the resulting ratio by 100. Necked nonwovens are generally extensible in the necked direction by an amount corresponding (but not a linear relationship) to the percent neckdown during necking. The extensibility of a necked nonwoven is measured herein as the percent elongation by elongating a necked nonwoven in the necked direction to the maximum extent possible without elongating individual fibers within the nonwoven, disrupting any fiber-to-fiber bonds within the nonwoven or tearing the nonwoven.

The term "easily extensible as-made nonwoven" is used herein to mean a nonwoven which, without any additional processing step (such as necking) beyond that normally used in the nonwoven production process, has a cross-direction elongation of at least 30% (typically about 60% to about 150%) without rupturing by application of a force of less than 200 grams per inch (g/in), typically less than 100 g/in, as

determined by the "Force Required to Elongate to 30%" method described in the Test Method section. An elongation of 50% means that a 10-inch wide sample can be elongated to 15 inches. Examples of suitable easily extensible as-made nonwovens may have a basis weight between about 15 to about 100 grams per square meter ( $\text{g}/\text{m}^2$ ), typically about 30 to about 80  $\text{g}/\text{m}^2$ , and a machine direction break tenacity of greater than 500  $\text{g}/\text{in}$  as determined by the "Break Tenacity Analysis" described in the Test Method section. Easily extensible as-made nonwovens can be spunlaced (also referred to as hydroentangled), melt blown, or thermally-bonded nonwovens and can be made by these well-known processes.

The term "spunlaced nonwoven" is used herein to refer to a fabric which has been formed by impinging a web (which can include preformed fabrics, spunmelt webs, air laid webs and carded webs) or a batt with jets of high pressure water. Easily extensible as-made nonwovens include Type 8075 Sontara® (Sontara® is a registered trademark of E.I. DuPont de Nemours and Company) and Flat Type Spunlaced Nonwoven, Item Number 4055-T produced by Sheng Hung Industrial Company, Taipei, Taiwan.

The term "melt blown nonwoven" is used herein to refer to a nonwoven formed by extruding molten polymer through a die into a high velocity stream of hot air or steam which converts the resulting filaments into fine and relatively short fibers. The fibers are deposited on a moving screen or belt and subsequently consolidated by a calendering, embossing, heated air, or other thermal bonding process.

The term "thermally-bonded nonwoven" is used herein to refer to a fabric composed of a web or batt of fibers which contains heat-sensitive material, such as specially engineered low-melting-point binder fibers or a thermoplastic powder having a melting point less than the web fiber, which melts and adhesively bonds the fibers of the web or batt into a consolidated nonwoven upon the application of heat, for example by hot air, calendering, embossing, infrared heat, or other thermal bonding process, with or without pressure.

The term "nonwoven substrate" is used herein to refer to a substrate which can be either a necked nonwoven substrate or an easily extensible as-made nonwoven substrate.

The term "nonwoven fabric" is used herein to refer to a fabric which can be either a necked nonwoven fabric or an easily extensible as-made nonwoven fabric.

The term "substantially uniformly impregnating" or "substantially uniformly impregnated" as used here refers to distributing a treatment or solution evenly through a bulk volume.

The term "wet coagulation" is used herein to describe a process in which a nonwoven substrate, having impregnated therein a solution comprising an elastomeric polymer dissolved in a solvent, is contacted with a coagulating liquid which is a non-solvent for the elastomeric polymer but is miscible with the solvent used to form the elastomeric polymer solution. The coagulating liquid is also selected such that it does not dissolve the nonwoven substrate. The coagulating liquid causes the polymeric material to be coagulated and the solvent to be removed into the coagulating liquid. The coagulating liquid is subsequently removed from the polymer-impregnated nonwoven, such as by air drying or heating.

Neckable nonwoven fabrics suitable for use in the current invention include spunbond webs, bonded carded webs, and hydroentangled webs. The neckable nonwoven fabric is preferably typically necked in the cross-direction using methods known in the art to achieve a percent neckdown of between about 25% and about 75% to obtain a necked nonwoven substrate having a percent elongation in the cross-direction of between about 30% and about 300%. Neckable nonwoven

fabrics useful in the current invention may be made from a number of thermoplastic polymers including nonelastomeric polyolefins such as polyethylene, polypropylene, ethylene copolymers, polyamides, polyesters, polystyrene, and poly-4-methylpentene-1. For example, the neckable nonwoven fabric comprises polypropylene, polyester, or a polypropylene-polyethylene copolymer. In a preferred embodiment, the neckable nonwoven fabric is a spunbond polypropylene fabric or carded thermal bond polypropylene or polyester fabric. 10 The starting neckable nonwoven substrate preferably typically has a basis weight between about 10  $\text{g}/\text{m}^2$  and about 50  $\text{g}/\text{m}^2$ . Relatively low basis weight neckable nonwovens are especially preferred such as those having a basis weight between about 10  $\text{g}/\text{m}^2$  and about 20-30  $\text{g}/\text{m}^2$ . The nonwoven substrate is typically moisture vapor permeable. The neckable nonwoven substrates are necked to provide necked nonwoven substrates generally having a basis weight greater than about 15  $\text{g}/\text{m}^2$ .

Necked nonwoven fabrics are known in the art and are 20 generally prepared by elongating a neckable nonwoven fabric in the machine direction to provide a necked nonwoven fabric that is necked in the cross-direction. Examples of necking processes are disclosed, for example, in U.S. Pat. No. 4,443, 513 to Meitner et al. (Meitner), U.S. Pat. Nos. 4,965,122, 25 4,981,747, and 5,114,781 (all to Morman). A preferred necking process is disclosed in U.S. Re 35,206 to Hassenboehler Jr. et al. (Hassenboehler). U.S. Re 35,206 is a reissue of U.S. Pat. No. 5,244,482 and is hereby incorporated by reference. A 30 nonwoven web that has been necked according to the process of Hassenboehler is also referred to herein as a "consolidated web".

Necked nonwovens can be prepared using relatively low 35 cost processes and are preferred over other extensible nonwoven fabrics because they have a higher degree of cross-direction extensibility and require relatively low extension (load) forces to extend the nonwoven in the cross-direction. In addition, necked nonwoven fabrics are generally substantially inextensible in the machine direction, that is they have a percent elongation of less than about 10% when subjected to 40 a biasing force in the machine direction. Stretch in substantially one direction is highly desirable in certain end uses as discussed below.

In a preferred embodiment, the necked nonwoven substrate 45 is a consolidated web prepared using the method described in Hassenboehler. This method involves passing a bonded thermoplastic nonwoven web having relatively low processing extensibility through a heated zone, such as an oven, to increase the temperature of the web to a temperature between the polymeric web's softening temperature and melting temperature while drawing the web in the machine direction thereby plastically deforming the fibers oriented in the cross-direction and consolidating (necking) the web in the cross-direction. The drawing is conducted by passing the web into the zone at a first linear velocity and withdrawing it at a 55 second linear velocity that exceeds the first velocity. The ratio of the second velocity to the first velocity is for example in the range from about 1.1:1 to about 2:1. The starting bonded nonwoven web is a non-elastomeric neckable nonwoven fabric and is selected to have a breaking draw ratio during hot 60 processing of less than about 4.0:1 and greater than about 1.4:1 evaluated while hot drawing at a strain rate greater than 2500%/min and a temperature greater than the softening point, but at least 10° F. less than the melting temperature of the polymeric web. The room temperature elongation (strain) 65 at break is for example between 2 and 40 percent, typically between 5 and 20 percent, based on test method ASTM D 1117-77 using an Instron tensile testing machine.

The fibers in the starting web may be bonded by fiber-to-fiber fusion, fiber entanglement, or thermal bonds such as by point bonding. Typically, the fibers in the neckable nonwoven fabric have small average fiber diameters, for example less than about 50 micrometers. The bonding in the spunbond precursor is typically strong (e.g. high temperature point bonding) in order to locally elongate, buckle, and bend the filament segments without affecting the web integrity. In point bonding, the bond points and bonding pattern are generally selected such that the area of the bonding points is between about 5 and about 25% of the web area. The shape of the bonding points can be diamond shaped or a number of other shapes well known in the art.

The heated drawing step causes plastic deformation of the cross-direction fibers and consolidation of the web such that a majority of the fibers are aligned generally in the direction of draw (machine direction). The web is consolidated in the cross-direction as it is longitudinally elongated and heat set with respect to the starting nonwoven.

Necked nonwoven substrates having an elongation in the cross-direction of at least 30%, for example at least 50% can be used to prepare the elastic nonwoven sheet of the current invention. The percent neckdown of the nonwoven web during the consolidation process is for example between about 50% and about 75%, typically between about 60% and 70%, corresponding to an extensibility between about 100% and 300%, and 150% and 250%, respectively.

The basis weight of the necked nonwoven web can be 3 times or more higher than the basis weight of the starting neckable nonwoven web. The basis weight of the necked web is between about 15 g/m<sup>2</sup> and about 100 g/m<sup>2</sup>, for example between about 20 g/m<sup>2</sup> and about 100 g/m<sup>2</sup>, and typically between about 25 g/m<sup>2</sup> and about 100 g/m<sup>2</sup>. The basis weight of the necked nonwoven substrate is chosen according to the desired end use. For example, when used as elastic interliners the basis weight of the necked nonwoven is typically between about 30 g/m<sup>2</sup> and 70 g/m<sup>2</sup> whereas for hygiene end uses such as diaper waistbands, etc. the basis weight is typically between about 15 g/m<sup>2</sup> and 40 g/m<sup>2</sup>. The basis weight of the necked nonwoven substrate should also be selected to achieve the desired elasticity in the final impregnated nonwoven. Higher basis weight nonwoven substrates allow more elastomeric polymer to be impregnated into the nonwoven, increasing the unload force of the impregnated nonwoven sheet.

Use of relatively low basis weight nonwovens in the necking process described in Hassenboehler is preferred for preparing materials made according to this invention. Used together, and after impregnation with an elastomeric polymer, these factors combine to provide stretchable nonwovens with a relatively low force required to extend the material (load force) and a relatively high retractive force exerted by the material as it is allowed to relax (unload force). This characteristic is preferred for end uses envisioned for this material. The relationship of unload force to load force is related to the hysteresis of the elastic nonwoven. For the preferred products of the current invention, having a cross-direction percent elongation of at least 150%, the ratio of the unload force at 100% elongation to the load force at 100% elongation, after the impregnated nonwoven has been extended to 140% three times and allowed to relax between extensions, is at least 0.3:1 and for example greater than 0.45:1.

Elastomeric polymers useful in this invention include polyurethanes, styrene-butadiene block copolymers, and polyether-ester block copolymers. In a preferred embodiment, the elastomeric polymer is a polyurethane.

Elastomeric polyurethanes useful in this invention can be prepared by reacting a polymeric glycol with a diisocyanate

to form a capped glycol, dissolving the capped glycol (in a suitable solvent), and then reacting the capped glycol with a difunctional chain extender having active hydrogen atoms. Such polyurethanes are termed "segmented" because they are comprised of "hard" urethane and urea segments derived from the diisocyanate and chain extender and "soft" segments derived primarily from the polymeric glycol. Suitable solvents for preparing solutions of such polymers are amide solvents such as dimethylacetamide ("DMAc"), dimethylformamide ("DMF"), and N-methyl-pyrrolidone, but other solvents such as dimethylsulfoxide and tetramethylurea can also be used.

Polymeric glycols used in the preparation of the elastomeric polyurethanes include polyether glycols, polyester glycols, polycarbonate glycols and copolymers thereof. Examples of such glycols include poly(ethyleneether) glycol, poly(tetramethyleneether) glycol, poly(tetramethylene-co-2-methyl-tetramethyleneether) glycol, poly(ethylene-co-butylene adipate) glycol, poly(2,2-dimethyl-1,3-propylene dodecanoate) glycol, poly(pentane-1,5-carbonate) glycol, and poly(hexane-1,6-carbonate) glycol.

Useful diisocyanates include 1-isocyanato-4-[(4-isocyanato-phenyl)methyl]benzene, 1-isocyanato-2-[(4-isocyanato-phenyl)methyl]benzene, isophorone diisocyanate, 1,6-hexanediiisocyanate, and 2,4-tolylene diisocyanate.

The chain extender can be a diol or a diamine. Useful diols include ethylene glycol, 1,3-trimethylene glycol, 1,4-butanediol, and mixtures thereof. Use of diol chain extenders leads to polyurethanes. Useful diamines include ethylene diamine, 1,2-propanediamine, 2-methyl-1,5-pentanediamine, 1,3-diaminopentane, 1,4-cyclohexane-diamine, 1,3-cyclohexanediamine, and mixtures thereof. In this case, the polymer produced is a polyurethaneurea (a sub-class of polyurethanes). When a polyether glycol and a diamine chain extender are utilized, the polymer produced is a polyetherurethaneurea; when a polyester glycol is utilized in combination with a diamine chain extender, a polyetherurethaneurea is produced. Monofunctional amine chain terminators such as diethyl amine, butylamine, cyclohexylamine, and the like can be added to control the molecular weight of the polymer. In a preferred embodiment, the elastomeric polymer is a diamine-extended polyurethane elastomer.

Solvents suitable for preparing the elastomeric polymer solutions include dimethylacetamide, dimethylformamide, and N-methyl-pyrrolidone. The viscosity of the elastomeric polymer solution is directly related to the concentration of the polymeric material in solution and consequently, the solution viscosity can influence both the degree of penetration of the polymer into the necked nonwoven fabric or the easily extensible as-made nonwoven fabric and the amount of polymer deposited therein. When the solution viscosity is too low, insufficient amounts of elastomer may be deposited in the necked nonwoven substrate or in the easily extensible as-made nonwoven substrate resulting in low unload force. When the solution viscosity is too high, penetration of the solution into the nonwoven substrate may be reduced, thereby resulting in incomplete or nonuniform impregnation of the polymer into the nonwoven substrate or formation of a layer of the polymer on the surface of the nonwoven substrate. The solution of elastomeric polymer to be impregnated into the necked nonwoven substrate or the easily extensible as-made nonwoven substrate for example has a solution viscosity of approximately 1000-300,000 centipoise ("cPs"), typically 10,000-40,000 cPs, measured at 25° C. The solution can comprise about 5 wt % to 20 wt % polymer.

It is necessary that the necked nonwoven substrate or the easily extensible as-made nonwoven substrate is able to

absorb the polymer solution and that the polymer solution substantially completely and uniformly impregnate the nonwoven substrate. The necked nonwoven substrate or the easily extensible as-made nonwoven substrate should therefore not be coated or otherwise treated in such a way as to prevent the polymer solution from being absorbed into the necked nonwoven fabric or the easily extensible as-made nonwoven fabric. The elastomeric polymer solution and/or the nonwoven fabric can include a surface-active agent to facilitate the impregnation of the web by the polymeric solution. Suitable surface-active agents include non-ionic wetting agents such as polymeric surfactants.

Additives, for example, pigments, antioxidants, ultraviolet light stabilizers and lubricants, can be added in small quantities to the elastomeric polymer solution, provided such additives do not detract from the benefits of the invention.

The elastomeric polymer solution may contain dispersed therein very short, fine fibers, such as cellulose fibers from wood pulp, cotton dust, or other synthetic or natural fibers having a length less than about 0.10 inches (2.5 mm), for example less than 0.5 mm. The fibers are typically small enough to fully penetrate the nonwoven fabric during the impregnation step. The short fibers can be added to the polymeric solution in amounts sufficient to deposit between about 3 and about 12 weight percent of short fibers in the impregnated nonwoven sheet, calculated based on the total weight of the nonwoven/elastomeric polymer composite. The short fibers are typically added to the elastomeric polymer solution at between about 10 and about 30 weight percent, for example between about 10 and about 20 weight percent, based on the total weight of the short fibers, elastomeric polymer, and solvent. Nonwoven sheets of the invention which have been prepared by impregnating a necked nonwoven fabric or an easily extensible as-made nonwoven fabric with an elastomeric polymer solution containing powdered cellulose may have a softer hand than those prepared using impregnating solutions which do not contain short fibers. An example of a very fine fiber particulate material suitable for use in the polymer solutions is powdered cellulose available under the trade name "Arbocel 30" available from J. Rettenmaier USA (Schoolcraft, Mich.).

Any suitable method of coating the elastomeric polymer solution onto the necked nonwoven substrate or the easily extensible as-made nonwoven substrate or otherwise impregnating the necked nonwoven substrate or the easily extensible as-made nonwoven substrate can be used as long as the fabric is uniformly impregnated and the coating is not concentrated on one or the other surface of the necked nonwoven substrate or the easily extensible as-made nonwoven substrate. It should be noted that, although coating methods may be employed to treat the nonwoven substrate with the elastomeric polymer solution, the solution and nonwoven properties and the coating process conditions are selected such that the polymer solution completely wets the nonwoven substrate or is otherwise completely absorbed into or driven into the nonwoven substrate so that a polymeric layer is not formed on either surface of the nonwoven substrate. In general, the amount of polymeric solution applied during coating can be controlled by utilizing a coating implement held at a predetermined distance above the necked nonwoven fabric or the easily extensible as-made nonwoven substrate. The solution can also be mechanically pressed into the nonwoven substrate. Rollers, platens, scrapers, knives, and the like can be used in the process of this invention as coating implements. Spraying the solution onto the nonwoven substrate can also be effective provided that the elastomeric solution substantially completely and uniformly impregnates the nonwoven

substrate. The force of the spray can be adjusted to assist in obtaining good penetration. The nonwoven substrate may be impregnated with the elastomeric polymer solution using a process known in the art as a "dip and squeeze" method in which the fibrous web is dipped or otherwise immersed into a tank containing the elastomeric polymer solution followed by squeezing, such as between nip rolls, to remove excess polymer solution. This method is preferred in order to minimize differences between the two surfaces of the stretchable composite nonwoven sheet.

The necked nonwoven substrate or the easily extensible as-made nonwoven substrate is impregnated with sufficient polymer solution to provide the desired unload/load force ratio in the final impregnated nonwoven sheet. The nonwoven substrate is typically impregnated with sufficient polymer solution to deposit therein between about 10 and about 80 weight percent elastomeric polymer, for example between about 30 and about 50 weight percent of elastomeric polymer, based on the total weight of elastomeric polymer and nonwoven substrate. When the amount of elastomer is too low, the ratio of unload force to load force can be undesirably low, and when the amount of elastomer is too high, the hand of the surfaces of the sheet can be undesirably tacky. The solution concentration and/or the amount of solution impregnated into the necked nonwoven fabric or the easily extensible as-made nonwoven substrate can be adjusted to achieve the desired polymer content in the impregnated sheet. For example, it was observed that using lower polymer concentration in the solution while retaining a similar elastomer content on the impregnated sheet by using a wider gap between nip rolls during application of the solution gave a product having an improved balance of hand and unload/load force ratio.

Once the nonwoven substrate has been impregnated with a solution comprising a solvent and an elastomeric polymer, the solvent is removed. The solvent is removed by wet coagulation followed by removal of the coagulating liquid. Wet coagulation provides a product having a surprisingly softer, more cloth-like hand than thermal drying. Wet coagulation processes are well known in the art and are commonly used in the production of artificial leathers. Water is preferred as the coagulating liquid due to ease of handling and low cost. Other suitable coagulating liquids include methanol, ethanol, isopropanol, acetone, or methylethyl ketone. A solvent for the elastomeric polymer such as dimethylformamide, dimethylacetamide, or N-methyl-pyrrolidone or other additives such as surfactants may be added to the coagulating liquid to modify the rate of coagulation. In addition, the temperature of the coagulation bath can be controlled to change the coagulation rate. Slower coagulation rates give the impregnated nonwoven a more attractive hand after the solvent has been removed.

In the impregnated nonwoven sheet of the current invention, the elastomeric polymer phase uniformly distributed throughout the necked nonwoven substrate or the easily extensible as-made nonwoven substrate is breathable. Also, the impregnated nonwoven sheet is typically moisture vapor permeable.

The hand of the impregnated nonwoven sheet can be improved by sanding or napping to raise fibers on the surface of the impregnated sheet resulting in a softer hand. Napping involves passing a fabric over a rotating roll that contains small metal points that effectively brush the fabric to raise fibers to the surface. In sanding, the metal brush is replaced with a rotating roll coated with sandpaper. Typically, the impregnated fabric is napped or sanded on both surfaces. For example, the fabric can be sanded with 80 to 200 grit sandpaper.

## 11

The stretchable impregnated nonwoven sheets of the current invention typically have a basis weight between about 40 g/m<sup>2</sup> and about 100 g/m<sup>2</sup>. They are especially useful in the waistbands or side panels of diapers and other personal hygiene garments such as underwear. Diapers are assembled commercially on long, high-speed lines in which the various diaper components are typically added in the machine direction to avoid slowing of the process. This is particularly true of elastomeric materials, which are normally stretched prior to insertion. A diaper generally includes about 20 or more individual components which must all be placed precisely in the right location on the diaper during the high-speed manufacturing process. This is much easier to achieve if the component (tape, sheet, fiber, etc.) is fed in the same direction in which the diaper is moving. To add components in the cross-direction (e.g. a waistband), it is preferable that the material itself stretches in the cross-direction so that it can be fed into the diaper making process as a tape in the machine direction. For example, this tape may be a 7 inch wide and only 1 inch long piece that is cut from a sheet and glued to a diaper or other disposable undergarment. In such processes, it is also preferred that the diaper component being fed into the process be substantially inextensible in the machine direction to facilitate feeding into the process. The stretchable nonwoven sheets of the current invention are substantially inextensible in the machine direction and have a high degree of recoverable stretch in the cross-direction, making them particularly suitable for use in such a process.

The stretchable nonwoven sheets of the current invention are also useful as an elastic interliner for various garments, particularly in jackets and coats. Interliners are fabrics inserted between the outer and inner layers of a garment that are intended to impart or to improve shape retention, padding, insulating value, stiffening, or bulk to a garment. The stretch nonwoven sheets of the current invention are particularly useful for this application because of their low cost combined with permanent elasticity and the ability to provide stretch for comfort in the around-the-body dimension.

## Test Methods

## Force Required to Elongate to 30%

This analysis was performed on an Instron Model 5565 equipped with the Merlin data collection software system. Both the Merlin system and instrument hardware are available from Instron Corporation (Braintree, Mass.). A one inch +/-0.05 inch wide (2.54 cm +/-0.13 cm) and approximately 8 inch (20.32 cm) long sample of a nonwoven sheet is clamped in the jaws of the Instron machine with a sample length set at 3.00 inches (7.62 cm). The sample is prepared such that the length of the sample is aligned with the cross-direction of the nonwoven. The sample is elongated at a rate of six inches per minute (15.24 cm/min) to an elongation of 30%. The force in grams at 50% elongation is recorded.

## Break Tenacity Analysis

This analysis was performed on an Instron Model 5565 equipped with the Merlin data collection software system. Both the Merlin system and instrument hardware are available from Instron Corporation (Braintree, Mass.). A one inch +/-0.05 inch wide (2.54 cm +/-0.13 cm) and approximately 8 inch (20.32 cm) long sample of a nonwoven sheet is clamped in the jaws of the Instron machine with a sample length set at 3.00 inches (7.62 cm). The sample is prepared such that the length of the sample is aligned with the cross-direction of the nonwoven. The sample is elongated at a rate of six inches per

## 12

minute (15.24 cm/min) until the sample breaks into two portions and the maximum force in grams at the break point is recorded.

## Basis Weight

A rectangular sample of nonwoven sheet approximately 1.0 inch by 8.0 inches (2.54 cm by 20.32 cm) is relaxed with care so that the sample contains no puckers or wrinkles. The length and width of the sample are measured to the nearest millimeter and the sample is weighed to the nearest tenth of a milligram. The weight is divided by the calculated area and the result expressed in terms of grams per square meter to the nearest 0.1 gram.

## Load and Unload Force Analysis

This analysis was performed on an Instron Model 5565 equipped with the Merlin data collection software system. Both the Merlin system and instrument hardware are available from Instron Corporation (Braintree, Mass.). A one inch +/-0.05 inch wide (2.54 cm +/-0.13 cm) and approximately 8 inch (20.32 cm) long sample of a nonwoven sheet is clamped in the jaws of the Instron machine with a sample length set at 3.00 inches (7.62 cm). The sample is prepared such that the length of the sample is aligned with the cross-direction of the nonwoven. The sample is elongated at a rate of six inches per minute (15.24 cm/min) to an elongation of 140% and then relaxed to its original length. This is repeated two more times and on the third cycle the force exerted by the material on the extension cycle (Load Force) is recorded at 50%, 100% and 135% elongation based on the original sample length and similarly, the force exerted by the material on the third relaxation cycle (Unload Force) is also recorded at the same elongation points. Results are expressed as Third Cycle Load and Unload forces, in grams, at the appropriate percent elongation.

## Percent Elongation Analysis

A relaxed strip of nonwoven fabric 1.0 inch (2.54 cm) wide and approximately 8 inches (20.32 cm) long that is free of puckers or wrinkles is marked with a pen at two points 4.0 inches (10.2 cm) apart such that the marks are approximately equal distance from the ends of the fabric. The ends of the fabric are then firmly held by the thumb and forefinger of each hand and the sample is fully extended, but not extended so far that the sample is torn or suffers any similar mechanical damage. The point of maximum elongation is apparent to the person performing the test as a noticeable increase in resistance to extension by the fabric. The length between the two marked points on the nonwoven is then measured and the percent elongation calculated by the following formula, where the initial length is 10.2 cm:

$$\text{Percent Elongation} = \left\{ \frac{(\text{elongated length} - \text{initial length})}{\text{initial length}} \right\} \times 100\%$$

When the percent elongation is measured in the necked direction, the fabric sample is cut with the length aligned with the cross-direction (necked direction).

## Example 1

A 30 inch (76.2 cm) wide, 15 g/m<sup>2</sup> wettable spunbond polypropylene nonwoven manufactured by Avgol Nonwovens, Israel, was fed through a nip roll at 89 feet per minute (27 m/min) and passed through a 72 inch (1.83 m) long forced air oven at 290° F. (143° C.) to a second nip roll operating at 115 feet per minute (35 m/min) and then onto a take up roll. In this process, the 30 inch (76.2 cm) wide nonwoven was uniformly and smoothly consolidated ("necked") in the cross-direction to a width of 10 inches (25.4 cm). It could be extended back to its original 30 inch (76.2 cm) cross-directional width by

13

application of minimal force. The necked nonwoven had essentially zero machine direction elongation and a basis weight of 32.0 g/m<sup>2</sup>.

The necked nonwoven was coated on one surface with a 15 mil (0.38 mm) doctor knife and a dimethylacetamide (DMAC) solution of 20% by weight of a polyurethaneurea derived from 1800 molecular weight poly(tetramethyleneether) glycol, 1-isocyanato-4-[(4-isocyanatophenyl)methyl]benzene (1.69 mole ratio of diisocyanate to glycol), chain extenders (ethylene diamine and 2-methyl-1,5-pentanediamine in a 9:1 mole ratio), and diethylamine. The following additives were also used: 0.5 wt % of a polymer of bis(4-isocyanatocyclohexyl)methane and (3-t-butyl-3-aza-1,5-pentanediol) (Methacrol® 2462B, a registered trademark of E. I. du Pont de Nemours and Company), 0.3 wt % titanium dioxide, 0.6 wt % silicone oil, 1.4 wt % 2,4,6-tris(2,6-dimethyl-4-t-butyl-3-hydroxybenzyl)isocyanurate (Cyanox® 1790, a registered trademark of Cytec Industries), and 4 wt % of a mixture of huntite and hydromagnesite. (All percentages based on polyurethaneurea weight.) The polyurethaneurea-DMAC solution fully wet the nonwoven.

The coated nonwoven was suspended substantially vertically in air for approximately 1 minute to allow full penetration of the polymer solution into the nonwoven and then immersed in a 70° F. (21° C.) bath of 40% by volume DMAC in water. After one minute, the impregnated fabric was successively transferred to 30 volume %, 20 volume % and 10 volume % DMAC/water solutions for one minute each and finally immersed in a 100% water bath for 2 minutes. The impregnated fabric was dried in air at room temperature.

The resulting impregnated nonwoven sheet had equivalent (dry, textile-like) hand and texture on both surfaces. Photomicrographs of the cross-section of the impregnated nonwoven sheet indicated a uniform composite structure through the thickness of the material and substantially no areas of continuous polyurethane on either surface.

The nonwoven sheet was then lightly sanded with a 220 grit sand paper. The resulting material had a noticeably softer feel and visual observation showed numerous individual short fibers projecting from the surface compared to a completely smooth surface with no projecting fibers prior to sanding. It was unexpected that this treatment succeeded in giving a softer hand without significantly impairing the visual aesthetics or the elastic characteristics of the sheet.

The resulting impregnated nonwoven sheet had a basis weight of 71.4 g/m<sup>2</sup>, indicating a polyurethaneurea content of 39.4 grams per square meter, or approximately 55 weight % elastomeric polymer.

Hand elongation of the resulting material in the cross-direction indicated an elongation of between about 160% and 180%.

Load and Unload Force analysis gave the following results:

| Third Load Cycle Force |                     |
|------------------------|---------------------|
| % Elongation           | Load force in grams |
| 50                     | 67.3                |
| 100                    | 211.2               |
| 135                    | 409.7               |

14

| Third Unload Cycle Force |                       |  |
|--------------------------|-----------------------|--|
| % Elongation             | Unload force in grams |  |
| 50                       | 22.7                  |  |
| 100                      | 114.7                 |  |
| 135                      | 340.7                 |  |

Comparison of the data in the tables indicates that the ratio of unload force to load force at 100% elongation was 0.54.

### Example 2

A portion, approximately 30 feet in length, of a 10 inch (25.4 cm) wide roll of a 55 g/m<sup>2</sup> flat type spunlaced nonwoven, Item Number 4055-T, manufactured by Sheng Hung Industrial Co., 116 Hou Kang Street, Shih-Lin District, Taipei, Taiwan, ROC, was used for this Example, which was run in a continuous fashion. The nonwoven substrate was first impregnated by immersion in a T-162 Lycra(R) solution in dimethylacetamide (DMAC) which contained 12.5% solids, which is available from INVISTA Inc., Wilmington, Del. Fabric speed was 3 ft/min with total fabric length in the bath being about 6 inches. Removal of excess polymer solution was accomplished by passing the impregnated fabric through a nip roll with a gap of 0.007 inches.

The resulting impregnated fabric was then passed through a bath of 40% DMAC dissolved in water, followed by two separate baths of 100% water. The fabric speed through these baths was 3 ft/min. The total fabric length in each bath was 8 feet. All baths were operated at room temperature, approximately 72° F. (40° C.). The resulting fabric was air dried to yield a breathable stretch nonwoven with attractive elastic properties and a basis weight of 80 g/m<sup>2</sup> (45% by weight T-162 Lycra(R)).

Hand Percent Elongation Analysis of the resulting elastic nonwoven in the cross-direction indicated an elongation of between 50% and 60%. Load and unload force analysis on the third cycle was performed as described in the Test Method section except that the sample was elongated to a maximum elongation of 50% and the load and unload retractive forces were recorded at 20%, 30%, and 40% elongation. This modified load and unload force analysis gave the following results:

| Third Load Cycle Force |                     |
|------------------------|---------------------|
| % Elongation           | Load force in grams |
| 20                     | 92.6                |
| 30                     | 227.2               |
| 40                     | 425.9               |

| Third Unload Cycle Force |                       |
|--------------------------|-----------------------|
| % Elongation             | Unload force in grams |
| 20                       | 20.0                  |
| 30                       | 75.9                  |
| 40                       | 192.0                 |

Comparison of the data in the tables indicates that the ratio of unload force to load force at 30% elongation was 0.33.

**15**

What is claimed is:

1. A stretchable nonwoven sheet consisting of a necked nonwoven substrate substantially uniformly impregnated with an elastomeric polymer solution without forming an elastomeric polymer layer on either surface of said substrate, the stretchable nonwoven sheet having a ratio of third unload cycle force at 100% elongation to third load cycle force at 100% elongation, after the stretchable nonwoven sheet has been extended to 140% in the necked direction three times, of at least 0.3:1, wherein the necked nonwoven substrate has a percent elongation in a cross-direction of between about 30% and about 300% and, wherein the stretchable nonwoven sheet has a thickness of 0.25 mm to 0.75 mm.

2. The stretchable nonwoven sheet according to claim 1 wherein the ratio of unload force to load force is at least 0.45:1.

3. The stretchable nonwoven sheet according to claim 1 wherein the sheet comprises about 10-80 weight percent of the elastomeric polymer based on the total weight of elastomeric polymer and nonwoven substrate.

4. The stretchable nonwoven sheet according to claim 1 wherein the nonwoven sheet has a basis weight between about 40 g/m<sup>2</sup> and about 100 g/m<sup>2</sup>.

5. A personal hygiene garment comprising the stretchable nonwoven sheet of claim 1.

6. A personal hygiene garment according to claim 5 wherein the garment comprises a diaper.

**16**

7. A personal hygiene garment according to claim 5 wherein the garment comprises underwear.

8. A garment comprising the stretchable nonwoven sheet of claim 1 wherein the stretchable nonwoven sheet is an interliner.

9. The stretchable nonwoven sheet according to claim 1 wherein the necked nonwoven substrate has a percent elongation in a cross-direction of between about 100% and about 300%.

10. The stretchable nonwoven sheet according to claim 1 wherein the necked nonwoven substrate has a basis weight between about 15 g/m<sup>2</sup> and about 100 g/m<sup>2</sup>.

11. The stretchable nonwoven sheet according to claim 1 wherein the necked nonwoven substrate has a basis weight between about 15 g/m<sup>2</sup> and about 40 g/m<sup>2</sup>.

12. The stretchable nonwoven sheet according to claim 1 wherein the necked nonwoven substrate has a basis weight between about 30 g/m<sup>2</sup> and about 70 g/m<sup>2</sup>.

13. The stretchable nonwoven sheet according to claim 1 wherein the sheet comprises between about 30 and about 50 weight percent of the elastomeric polymer based on the total weight of elastomeric polymer and nonwoven substrate.

14. The stretchable nonwoven sheet according to claim 1 wherein the elastomeric polymer solution contains dispersed therein fine fibers.

\* \* \* \* \*